# EUROPEAN PATENT SPECIFICATION

(11) **EP 2 578 804 B1**
(45) Date of publication and mention of the grant of the patent: **26.12.2018**
(21) Application number: 12186293.2
(22) Date of filing: 27.09.2012
(51) Int. Cl.: F01D 5/20, F01D 11/12

(54) **METHOD OF MANUFACTURING AN ABRADABLE AIR SEAL**
HERSTELLUNGSVERFAHREN EINER ABREIBBAREN SPALTDICHTUNG
PROCÉDÉ DE FABRICATION D'UN JOINT D'USURE ABRADABLE

(30) Priority: 20.09.2011 US 201113236926
(43) Date of publication of application: 10.04.2013
(73) Proprietor: United Technologies Corporation, Farmington, CT 06032 (US)
(72) Inventor: Strock, Christopher W., Kennebunk, ME Maine 04043 (US); Reynolds, George H., Sanford, ME Maine 04073 (US)
(74) Representative: Dehns

(56) References cited:
- EP-A1- 0 416 954
- EP-A1- 1 734 146
- EP-A1- 1 865 150
- EP-A1- 2 281 913
- WO-A1-2011/008719
- DE-A1-102007 047 739
- US-A1- 2004 142 196
- US-A1- 2005 124 505
- DIETER SPORER ET AL: "On the potential of metal and ceramic based abradables in turbine seal applications", INTERNET CITATION, 2007, pages 79-86, XP002660457, Retrieved from the Internet: URL:http://turbolab.tamu.edu/uploads/files /papers/t36/T36-LEC10.pdf [retrieved on 2013-02-20]

## Description

### BACKGROUND OF THE INVENTION

This disclosure relates to an air seal for a gas turbine engine.

In compressor and turbine sections of a gas turbine engine, air seals are used to seal the interface between rotating structure, such as a hub or a blade, and fixed structure, such as a housing or a stator. For example, typically, circumferentially arranged blade seal segments are fastened to a housing, for example, to provide the seal.

Relatively rotating components of a gas turbine engine are not perfectly cylindrical or coaxial with one another during engine operation. As a result, the relatively rotating components may occasionally rub against one another. To this end, an abradable material typically is adhered to the blade seal segments and/or the rotating component.

Document US 2004/0142196 A1 discloses a method of manufacturing an abradable layer using a thermal spray composition comprising a mixture of metal-clad hexagonal boron nitride hBN particles and unclad hBN particles. Document EP 2 281 913 A1 discloses a method of manufacturing an abradable layer comprising an oxide ceramic and hBN. An air seal with similar characteristics to the present invention is described in Dieter Sporer et al: "On the potential of metal and ceramic based abradables in turbine seal applications".

### SUMMARY

The present invention provides a method as set forth in claim 1.

### BRIEF DESCRIPTION OF THE DRAWINGS

Figure 1 shows a perspective view of a portion of a gas turbine engine incorporating an air seal.
Figure 2 shows a schematic view of an air seal.

### DETAILED DESCRIPTION OF THE PREFERRED EMBODIMENT

Figure 1 shows a portion of a gas turbine engine 10, for example, a high pressure compressor section. The engine 10 has blades 15 that are attached to a hub 20 that rotate about an axis 30. Stationary vanes 35 extend from a substrate 40, such as an outer case or housing, and are circumferentially interspersed between the turbine blades 15, which may be constructed from titanium in one example. A first gap 45 exists between the blades 15 and the substrate 40, and a second gap 50 exists between the vanes 35 and the hub 20.

Air seals 60 (Figure 2) are positioned in at least one of the first and second gaps 45, 50. Further, the air seals 60 may be positioned on: (a) the outer edge of the blades 15; (b) the inner edge of the vanes 35; (c) an outer surface of the hub 30 opposite the vanes 35; and/or (d) as shown in Figure 2, on the inner surface of outer case opposite the blades 15. It is desirable that the gaps 45, 50 be minimized and interaction between the blades 15, vanes 35 and seals 60 occur to minimize air flow around blade tips or vane tips. It should be recognized that the seal provided herein may be used in any of a compressor, a fan or a turbine section and that the seal may be provided on rotating or non-rotating structure.

In one example shown in Figure 2, the air seal 60 includes an abradable layer 70 supported on the substrate 40, which may be constructed from a nickel alloy, by a bond coat 65. The bond coat 65 may include a nickel alloy, platinum, gold, silver, or MCrAlY, wherein M includes at least one of nickel, cobalt, iron or a combination thereof.

The abradable layer consists of three ceramic materials, which have different material characteristics from one another, such as chemical composition and/or particle size. The abradable layer is a bimodal mix of a first ceramic material of an oxide ceramic (for example, stable up to at least 650°C (1200°F)) and second ceramic material of hexagonal boron nitride ("hBN"), and inclusions of a third ceramic material of larger hBN. No metallic material is used in the abradable layer, which greatly reduces its weight, for example, by around 30%. The abradable layer has a strength of at least 3.5 MPa (500 psi).

Feed stock used to provide the air seal 60 is made of oxide ceramic and hBN held together with a binder, plus hBN particles that are used at a variable ratio to the agglomerated composite powder to adjust and target the coating properties during manufacture.

The matrix of oxide ceramic and hexagonal boron nitride (hBN) includes hBN particles in the range 1-10 micron particle sizes and the oxide ceramic in the range of 1-45 micron particle size. Polyvinyl alcohol or bentonite may be used as a binder to agglomerate the oxide ceramic and hBN before thermal spraying. Larger particles of hBN are added to the fine composite matrix prior to spraying or during spraying. The larger hBN particles are in the range of 15-100 microns particle size, though 20-75 microns particle size may be typical.

The amount by volume of oxide ceramic in the abradable layer is about 25-45% with the matrix composite of oxide ceramic and hBN having a volume fraction of about 35-50% oxide ceramic. The amount by volume of porosity is about 5-15% of the abradable layer. The larger hBN particles make up the remainder of the coating, the total amount by volume of hBN in the abradable layer is 30-50% with up to 15% of the volume percent comprising the binder. In one example, the oxide ceramic is at least one of aluminum-, zirconium- and titanium-based.

In a first example, the oxide ceramic is a mix of aluminum oxide (Al₂O₃) and titanium dioxide (TiO₂). This titanium dioxide improves cracking and spallation resistance of the oxide ceramic. The mix includes 0-15% by weight of titanium dioxide. One desired mix is 87 wt% aluminum oxide/13 wt% titanium dioxide, and another desired mix is 97 wt% aluminum oxide/3 wt% titanium dioxide.

In a second example, the oxide ceramic includes about 7% by weight yttrium stabilized zirconia (YSZ).

The powders are deposited by a known thermal spray process, such as high velocity oxygen fuel spraying (HVOF), combustion flame spray or air plasma spray (APS). Fine particle-sized hBN powders and the fine particle-sized oxide ceramic powders being pre-agglomerated as described, are deposited on the substrate by thermal spray. The larger particle-sized hBN particles may be added to the agglomerates as a particle blend and delivered to the spray apparatus pre-blended, or may be delivered to the spray apparatus through a separate delivery system. However, it is also possible to include the larger hBN particles in the agglomerates of matrix material.

Typically, the matrix of agglomerated hBN powder and oxide ceramic powder and the larger hBN powder are fed into the plasma plume from separate powder feeders. The abradable layer 70 is deposited onto the substrate 40 (or bond coat 65) to a desired thickness, for example, 0.38-3.81 mm (15-150 mils), and in one example, 2.03 mm (80 mils).

Although an example embodiment has been disclosed, a worker of ordinary skill in this art would recognize that certain modifications would come within the scope of the claims. For that reason, the following claims should be studied to determine their true scope and content.

## Claims

1. A method of manufacturing a gas turbine engine air seal comprising:
depositing an abradable coating (70) onto a substrate (40), depositing the abradable coating (70) including:
agglomerating a matrix, and
mixing with the matrix a first hexagonal boron nitride powder;
**characterised in that** said matrix is agglomerated of a second hexagonal boron nitride powder and an oxide ceramic powder, wherein the amount by volume of oxide ceramic in the abradable layer (70) is about 25-45%, and the amount by volume of porosity is about 5-15% of the abradable layer (70), and wherein the second hexagonal boron nitride powder comprises particles of 1-10 microns agglomerated with the oxide ceramic powder which comprises particles of 1-45 microns, and the first hexagonal boron nitride powder comprises particles of 15-100 microns.

2. The method according to claim 1, wherein the oxide ceramic is a mix of aluminum oxide and titanium dioxide, and the mix includes 0-15% by weight of titanium dioxide.

3. The method according to claim 1, wherein the oxide ceramic includes about 7% by weight yttrium stabilized zirconia.

## Patentansprüche

1. Verfahren zur Herstellung einer Gasturbinenmotorspaltdichtung, das Folgendes umfasst:
Auftragen einer abreibbaren Beschichtung (70) auf ein Substrat (40), wobei das Auftragen der abreibbaren Beschichtung (70) Folgendes einschließt:
Agglomerieren einer Matrix,
Mischen der Matrix mit einem ersten hexagonalen Bornitridpulver;
**dadurch gekennzeichnet, dass** die Matrix aus einem zweiten hexagonalen Bornitridpulver und einem Oxidkeramikpulver agglomeriert wird, wobei die Volumenmenge der Oxidkeramik in der abreibbaren Schicht (70) etwa 25-45 % beträgt und die Volumenmenge an Porosität etwa 5-15 % der abreibbaren Schicht (70) beträgt, und wobei das zweite hexagonale Bornitridpulver Partikel von 1-10 Mikrometer umfasst, die mit dem Oxidkeramikpulver agglomeriert werden, das Partikel von 1-45 Mikrometer umfasst, und wobei das erste hexagonale Bornitridpulver Partikel von 15-100 Mikrometer umfasst.

2. Verfahren nach Anspruch 1, wobei die Oxidkeramik eine Mischung aus Aluminiumoxid und Titandioxid ist, und wobei die Mischung 0-15 Gew.-% Titandioxid einschließt.

3. Verfahren nach Anspruch 1, wobei die Oxidkeramik etwa 7 Gew.-% yttrium-stabilisiertes Zirkoniumdioxid einschließt.

## Revendications

1. Procédé de fabrication d'un joint d'usure de moteur à turbine à gaz comprenant :
le dépôt d'un revêtement abradable (70) sur un substrat (40), le dépôt du revêtement abradable (70) incluant :
l'agglomération d'une matrice, et
le mélange avec la matrice d'une première poudre de nitrure de bore hexagonal ;
**caractérisé en ce que** ladite matrice est agglomérée à une seconde poudre de nitrure de bore hexagonal et une poudre de céramique d'oxyde, dans lequel la quantité en volume de céramique d'oxyde dans la couche abradable (70) est d'environ 25-45 %, et la quantité en volume de porosité est d'environ 5-15 % de la couche abradable (70), et dans lequel la seconde poudre de nitrure de bore hexagonal comprend des particules de 1-10 microns agglomérés avec la poudre de céramique d'oxyde qui comprend des particules de 1-45 microns, et
la première poudre de nitrure de bore hexagonal comprend des particules de 15 à 100 microns.

2. Procédé selon la revendication 1, dans lequel la céramique d'oxyde est un mélange d'oxyde d'aluminium et de dioxyde de titane, et le mélange inclut de 0-15 % en poids de dioxyde de titane.

3. Procédé selon la revendication 1, dans lequel la céramique d'oxyde inclut environ 7 % en poids de zircone stabilisé par de l'yttrium.
